

E. G. GILSON.  
CURRENT COLLECTOR AND PROCESS OF MAKING THE SAME.  
APPLICATION FILED NOV. 17, 191  
Patented Mar. 10, 191  
1,089,700.

Fig.1.



Fig.2.



Witnesses:

Marcus L. Byng.  
J. W. Rice

Inventor  
Emery G. Gilson,  
by Alfred S. Davis  
His Attorney.

# UNITED STATES PATENT OFFICE.

EMERY G. GILSON, OF SCHENECTADY, NEW YORK, ASSIGNOR TO GENERAL ELECTRIC COMPANY, A CORPORATION OF NEW YORK.

## CURRENT-COLLECTOR AND PROCESS OF MAKING THE SAME.

1,089,700.

Specification of Letters Patent. Patented Mar. 10, 1914.

Application filed November 17, 1911. Serial No. 660,767.

To all whom it may concern:

Be it known that I, EMERY G. GILSON, a citizen of the United States, residing at Schenectady, county of Schenectady, State 5 of New York, have invented certain new and useful Improvements in Current-Collectors and the Process of Making the Same, of which the following is a specification.

My invention relates to brushes for dynamo electric machines, particularly to molded metal brushes, and it has for its object the provision of improved means for connecting the flexible conductors to such brushes.

15 Copper-graphite brushes, such as described in my previously filed application Serial Number 570,737, filed July 7th, 1910, are operated at a current density very much higher than the carbon brushes, that is 20 about 125 amperes per square inch under normal operating conditions. This necessitates very much better electrical connection between the flexible conductors and the brushes.

25 The flexible conductors ordinarily consist of a large number of fine wires or strands braided together. I have discovered that when these conductors are unbraided at their ends that these ramified ends may be 30 molded into the body of the brush and be caused to adhere so firmly to the metal particles in the brush as to become virtually a unitary part of the brush itself.

It is important that the final firing treatment to which the brush is subjected shall take place under conditions which will permit the conductors to retain their flexibility, and, therefore, I preferably fire the brushes in a vacuum.

40 For a better understanding of my invention, reference may be had to the following description taken in connection with the accompanying drawing in which—

Figure 1 is a perspective view of the 45 brush with flexible conductors attached to the brush by being molded therein; Fig. 2 is a sectional view showing the appearance of the ends of the conductors in the brush.

As described in my previously filed application above referred to, molded metallic brushes consisting of metal and graphite are manufactured by first making an intimate mixture of graphite and certain metallic oxids, preferably a copper oxid and an oxid

of a soft metal easily alloyable with copper, 55 such as tin oxid or lead oxid. This mixture is subjected to a reduction treatment which causes all but a small percentage of the metallic oxids to be reduced to the metallic state. The reduction takes place at 60 the expense of part of the graphite but I aim to leave about 4 to 12 per cent. of graphite in the mixture. It is also important that a few per cent. of oxid shall remain in the mixture. The reduced mixture 65 is molded into the form desired in the finished brush and is finally fired to consolidate the metal particles.

In accordance with my present invention, the unbraided ends of the flexible conductors are embedded in the metal-graphite mixture when it is being molded into the desired form. The brush with the embedded conductors is then fired in a vacuum or in the presence of a neutral gas or, in general, 75 in an environment which will not react chemically with the material of the conductor itself. I find that a reducing gas as was formerly commonly used to protect the brushes during the final firing treatment 80 exerts an unfavorable influence upon the flexible copper conductors so as to make them brittle. The individual strands also tend to adhere to each other and cause the conductor to become stiff. This effect is 85 probably due to the complete reduction of oxids in the copper.

The firing treatment may take place at a temperature of about 650° C. At this temperature, the particles of metal in the body 90 of the brush 2 attach themselves firmly to the individual wires or strands which make up the conductors 1. In my opinion this is due to the reduction of oxids in the strands and in the metal powder in immediate contact with the strands, and also to the formation of an alloy between the copper of the flexible conductors and the tin, lead or other soft metal in the brush mixture.

I find by this process that the mechanical 100 union between the flexible wires and the body of the brush is so intimate that the flexible conductors cannot be removed from the brush without partly or completely tearing the strands of the conductor itself. The 105 electrical contact under these conditions is of course far more perfect than any form of mechanical union.

What I claim as new and desire to secure by Letters Patent of the United States, is,

1. The process of connecting a pigtail to a molded current collector which consists in embedding the unstranded end of said pigtail in finely-divided metal, molding the same under pressure, and firing in an inert environment at a temperature sufficient to consolidate the metal particles.
- 10 2. The process of making current connections to molded metal brush which consists in embedding the end of a stranded conductor in the material of said brush in a finely-divided state, compressing said material and firing in a substantial vacuum at

a temperature at which said material will consolidate.

3. The process of making current connections to molded metal brush which consists in embedding the unbraided end of a 20 stranded conductor in finely-divided brush material containing some oxid, compressing said material and firing in a vacuum.

In witness whereof, I have hereunto set my hand this 15th day of November, 1911, 25

EMERY G. GILSON.

Witnesses:

HELEN ORFORD,  
BENJAMIN B. HULL.